

# UNITED STATES PATENT OFFICE.

WALTER FRANCIS REID, OF ADDLESTONE, ENGLAND, ASSIGNOR TO THE  
VELVRIL COMPANY, LIMITED, OF LONDON, ENGLAND.

## COVERING FOR DRAWING-ROLLS OF SPINNING MACHINERY.

SPECIFICATION forming part of Letters Patent No. 661,644, dated November 13, 1900.

Application filed February 6, 1900. Serial No. 4,269. (No model.)

*To all whom it may concern:*

Be it known that I, WALTER FRANCIS REID, civil engineer, a subject of the Queen of Great Britain, residing at Fieldside, Addlestone, in the county of Surrey, England, have invented certain new and useful Coverings Suitable for the Drawing-Rolls Used in Spinning, of which the following is a specification.

The drawing-rolls used in spinning cotton and other fibers are usually covered with tubes of leather; but such tubes are expensive and have the disadvantage of having a longitudinal seam. The leather also soon polishes and is grooved by the fibers, causing alterations in the tension of the thread. India-rubber and like compounds have been suggested, but are unsuitable, being acted upon by the grease in the cotton or other fiber.

According to this invention I employ a tube, preferably a seamless tube of a mixture of

nitrocellulose with nitroricinolein. A suitable mixture consists of one part, by weight, of nitrocellulose to two parts of nitroricinolein. Nitrolinolein is of precisely the same nature as nitroricinolein, and I wish to be understood as considering this as an equivalent. The tubes may be made in a variety of ways, such as by applying a solution of the mixture (in any of the usual solvents of nitrocellulose) to a revolving mandrel or by forcing the mixture under pressure through dies or by cementing together the edges of a street.

What I claim is—

A covering for the drawing-rolls used in spinning consisting of a mixture of nitrocellulose with nitroricinolein.

WALTER FRANCIS REID.

Witnesses:

VARASUN LARK,  
HENRY POPE.